

June 16, 1953

L. PORGES ET AL

2,642,230

PROCESS FOR DISTRIBUTING WAX IN CEMENTED CARBIDE POWDERS

Filed July 25, 1949



INVENTORS

LEO PORGES

STANLEY THOMAS SAWYER

By:

Hazeltine, Lake Co.

AGENTS

## UNITED STATES PATENT OFFICE

2,642,230

PROCESS FOR DISTRIBUTING WAX IN  
CEMENTED CARBIDE POWDERS

Leo Porges and Stanley T. Sawyer, London, England, assignors to A. Johnson &amp; Company (London) Limited, London, England

Application July 25, 1949, Serial No. 106,730  
In Great Britain February 25, 1948

2 Claims. (Cl. 241—15)

1

This invention relates to the mixing, milling and lubricating of finely divided metal powders and like pulverulent materials prior to pressing.

In the processing of metal powders it is usual, in current industrial practice, to place the constituent powders in a cylindrical container together with a suitable liquid such as distilled water, benzene, acetone or alcohol, which liquid promotes mixing and milling and prevents oxidation of the metal powders during milling, a number of balls being added to assist mixing and to increase the milling action. The container is sealed and fitted into a ball-milling machine and rotated for a certain period, usually varying between 24 and 120 hours. The liquid is then evaporated from the container and the powder, when dry, is separated from the balls and subjected to heat treatment in a reducing atmosphere to anneal the powder, since some powders become work-hardened during milling.

To disperse a small quantity of substance such as a lubricant uniformly throughout the metal powder the lubricant is dissolved in a solvent and then added to the powder, the liquid and the powder being mixed together in an "open pan" mixing machine, during which operation the solvent evaporates. When the bulk of the solvent has evaporated, the powder is finally dried in a drying oven. By this process the lubricant is not evenly distributed throughout the charge, some layers tending to have far more lubricant thereon than other layers.

Attempts have been made to distribute a lubricant throughout a finely divided powder by placing the powder in a container, adding the lubricant dissolved in a solvent thereto, and subjecting the container to a rotary movement. Satisfactory distribution of the lubricant has not been obtained by this method. The lubricated powder has a tendency to cake on the walls of the container, and if there are balls therein the powder will also cake around these. It must be emphasized that in this process the container is subjected to a rotatory movement.

According to the present invention there is provided a process for mixing and/or milling and uniformly distributing a comparatively small quantity of a substance throughout a finely divided material, wherein the finely divided material is placed in a container, and the substance which it is desired to distribute is dissolved in a solvent and added thereto, and wherein the container is subjected to a vibratory movement so that mixing and/or milling take place, the solvent being removed by heating and/or by application of a negative pressure before the termi-

2

nation of such vibratory mixing and/or milling.

The invention also includes any process containing the step of placing the finely divided material in a container and adding the substance, which it is desired to distribute, dissolved in a solvent thereto and then subjecting the container to a vibratory movement so that uniform distribution of the small quantity of substance takes place, the solvent being removed by heating and/or the application of a negative pressure before the termination of such vibratory movement.

For a better understanding of the invention, one mode of carrying it into effect will now be described with reference to the accompanying drawing, which shows a side-elevation, partly in section, of an apparatus which may be employed for carrying out the invention.

The mixing, milling lubricating and solvent distillation operations are carried out in a container 1, mounted on supporting plates 3, which are suspended by suspension rods 4 from the upper end of a framework 2, by angle-section supporting members 5. Supported within the framework 2, is an electric motor 6 which drives an eccentrically mounted flywheel within a casing 8 through a flexible coupling 7. The casing 8 imparts a vibratory motion to the plates 3 and hence to the container 1.

The container 1 is secured within an oil-jacket 9, the latter containing thermostatically controlled electric immersion heaters 10 inserted through a sealing lid 11. Additionally, the container 1 has a tightly fitting conical cover 12 with a flexible hose connection 13 which leads to a vacuum pump (not shown).

In the use of this apparatus, balls are placed in the container 1 and cemented carbide powder, together with a required quantity of wax dissolved in benzene is added thereto. The container 1 is then vibrated for a desired milling period and towards the end of this period the oil-jacket 9 is heated by the heaters 10, so that the solvent may be removed whilst the charge is still being vibrated. To accelerate the rate of evaporation and to reduce the possibility of oxidisation of the finely divided metal powder during the heating period, the container is subjected to a negative pressure through the hose connection 13.

The removal of the solvent by heating is not effected until the mixing and milling operation is almost completed. It is very important that the powder charge should be in a violent state of

agitation whilst this distillation is taking place, so that the lubricant will be uniformly distributed throughout the charge. When dry the container is emptied and the powder is separated from the balls, which are then returned to the apparatus.

It is found that metal powders prepared by this process do not become work-hardened, which means that there is no need for a subsequent heat treatment. This represents a saving both 10 of time and expense. It is, of course, known that the use of work-hardened powders gives rise to many difficulties in all the subsequent processing of such powders—for example, during the subsequent pressing and sintering operations. These processing difficulties exhibit themselves in one form or another, for example it may be difficult to press the final product or when it is so pressed cracks may develop therein.

It is also found that, with the product of the 20 invention, in the subsequent sintering process, even shrinkage of the product takes place in all three dimensions, that is, there is substantially an absence of distortion. This is because the lubricant has been evenly distributed throughout the charge and the particles thereof are hence uniformly lubricated. The pressed product has also a much more uniform porosity because of the even distribution of the lubricant.

While the invention has been described in its 25 application to the treatment of powder metals, it will be understood that it is equally applicable to a variety of other processes where it is desired to disperse a small quantity of a soluble solid body evenly throughout a comparatively 30 large quantity of finely divided material, e. g. in the manufacture of grinding wheels.

Further it should be noted that this invention is specifically suited to the mixing and/or milling and lubricating of cemented carbide powder 35 mixtures for subsequent processing into the final sintered state.

We claim:

1. A process for mixing, milling and uniformly distributing a comparatively small quantity of wax throughout finely divided cemented carbide pow-

ders, comprising the steps of placing finely divided cemented carbide powders in a container, dissolving the wax which it is desired to distribute in a solvent, adding the solution of said wax to said finely divided cemented carbide powders, grinding the powders by subjecting the powders in said solution to a violent vibration and evaporating said solvent during said violent vibration.

2. A process for mixing, milling and uniformly lubricating cemented carbide powders, comprising the steps of placing the cemented carbide powder in a container, dissolving wax in a solvent, adding the wax dissolved in the solvent to said cemented carbide powder, grinding the powders by subjecting the powders in said solution to a violent vibration and evaporating said solvent during said violent vibration.

LEO PORGES.  
STANLEY T. SAWYER.

References Cited in the file of this patent

UNITED STATES PATENTS

| Number    | Name   | Date          |
|-----------|--------|---------------|
| 1,920,234 | Arthur | Aug. 1, 1933  |
| 1,930,684 | Kramer | Oct. 17, 1933 |
| 2,002,891 | Hall   | May 28, 1935  |
| 2,272,629 | Arthur | Feb. 10, 1942 |

FOREIGN PATENTS

| Number  | Country       | Date          |
|---------|---------------|---------------|
| 376,242 | Great Britain | Jan. 1, 1931  |
| 593,777 | Great Britain | Oct. 24, 1947 |

OTHER REFERENCES

Noel et al. "Production and Some Testing Methods of Metal Powders." Transactions of American Institute of Mining and Metallurgical Engineers. Vol. 128 (1938), pp. 37-41, and 56. 83-94 (Metal).

Bachman, "Die Entwicklung der Schwingmühle," Chemische Technik, vol. 15, pages 195-204. September 5, 1942. 241/175.